

## UNITED STATES PATENT OFFICE

2,462,055

## BRUSH

Robert S. Herwig, North Arlington, N. J., assignor  
to Bendix Aviation Corporation, Teterboro,  
N. J., a corporation of Delaware

No Drawing. Application January 24, 1944,  
Serial No. 519,531

10 Claims. (CL. 171—325)

**1**  
The present invention relates to commutator and slip ring brushes for electrical devices and more particularly to a novel composition and method for producing a graphite or metal graphite brush for use in aircraft and having superior wearing qualities at high altitudes or under low moisture conditions.

As is well known, rapid wear or dusting of graphite or metal graphite brushes will occur when used on commutators or slip rings, if the moisture content of the air is reduced below a certain value which depends upon altitude, temperature and pressure.

It has been found that for the same water vapor concentration per cubic foot, the rate of wear increases as the atmospheric pressure surrounding the brushes decreases.

When brush wear occurs at a normal rate it has been found that the conventional copper commutator surface is covered by a layer of copper oxide over which is deposited a layer of carbon. When the oxide film is not maintained because of a reduction in the water vapor content of the surrounding atmosphere or the oxygen content is reduced below a density sufficient to maintain this oxide film rapid brush wear or dusting takes place. Thus it has been found that the presence of water vapor increases brush life by preventing dusting and the presence of oxygen increases the formation of films which also increase brush life by reducing the friction between the copper commutator and the graphite brush.

It is an object of my invention, therefore, to provide a brush, whereby both such optimum conditions for long wear may be obtained at high or low altitudes.

Another object of my invention is to provide a novel graphite brush mix, whereby the brush may be so impregnated as to provide such beneficial conditions.

Another object of my invention is to provide a porous brush for the adsorption of moisture and oxygen at low altitudes for use in preventing dusting at high altitudes.

Another object of my invention is to provide a mixture for the manufacture of graphite brushes including a reagent, which during a heating operation liberates a gas which increases the porosity of the brush and forms a hygroscopic oxide, whereby moisture vapor may be adsorbed by the brush through capillary action as well as by the hygroscopic nature of the oxide so as to prevent excessive wear of the brush at high altitudes.

**2**  
It is also an object of my invention to provide a commutator brush particularly adapted for use on an aircraft, and including an inorganic moisture adsorbent composition, whereby moisture vapors may be adsorbed by the brush when the aircraft is at altitude levels having an atmosphere containing a relatively high moisture content, so as to serve as a moisture supply for preventing the dusting of the brush at altitudes having an atmosphere containing a relatively low moisture content.

Other objects and advantages of this invention are set forth in the following description and the novel features thereof are pointed out in the appended claims. The disclosures, however, are illustrative only and changes may be made therein within the principle of the invention to the full extent indicated by the broad and general meanings of the terms in which the appended claims are expressed.

Specifically, as an example of my invention, a brush such as described may be readily formed by adding to a metal-graphite mixture, which may contain by weight 60% carbon and 40% copper, an amount of barium nitrate

$(Ba(NO_3)_2)$

equal to approximately 7% by weight of the metal-graphite mixture. The said ingredients may then be well mixed in any suitable manner and compressed or otherwise formed into a block of suitable size to form the commutator brush. The mixture may then be baked at approximately 1,500° F. by suitable heating means for a period sufficient to permit the barium nitrate to be converted by the heat treatment into a hygroscopic barium oxide ( $BaO$ ). The nitrogen gases thus liberated will activate the graphite mixture so that upon removal of the same from the heat treatment, there is formed a porous block. The porosity of the metal graphite block, thus formed, permits upon cooling and exposure to atmosphere, the atmospheric moisture vapors to be adsorbed by the block through a capillary action, as well as by the hygroscopic barium oxide ( $BaO$ ).

It has been found that the metal-graphite brush formed in the manner described has remarkable wearing qualities when used in an aircraft with the conventional copper commutators of electric motors, generators or other similar moving parts.

The long life of such graphite brushes is believed to be attributable to the barium nitrate being converted to a porous hygro-

scopic barium oxide (BaO) during the heat or baking process. Also the liberation of nitrogen gases during the heat treatment activates the graphite mixture resulting in a porous block structure. Since barium oxide (BaO) is extremely hygroscopic, moisture vapors are adsorbed into the brush at low altitudes where free moisture is prevalent so as to serve as a moisture supply for preventing the dusting or wearing of the brush due to lack of moisture at the extremely high altitudes.

The residual moisture carried by the brush serves to catalyze the formation of cuprous oxide (Cu<sub>2</sub>O) on the conventional copper commutator. As is well known cuprous oxide (Cu<sub>2</sub>O) when in contact with graphite becomes an excellent lubricant.

The porosity of the graphite increases the amount of water vapor that the brush would normally adsorb. The adsorbed water vapor is liberated at high altitude causing the brush to be cooled by evaporation and, further, escaping oxygen reduces the friction between the graphite and the copper commutator by oxidizing any raw copper surface.

While barium oxide (BaO) is hydroscopic it is only slightly water soluble so that after a flight at high altitude the brush is regenerated when the plane again returns to a level where moisture vapors are more prevalent as at sea level.

As another example of my invention I have found that by adding calcium sulfate dihydrate (CaSO<sub>4</sub>.2H<sub>2</sub>O) to a suitable metal graphite mixture and properly baking the same, similar superior wearing qualities may be obtained. Thus, for example, such a graphite brush may be formed by adding to a metal graphite mixture containing by weight 60% carbon and 40% copper an amount of calcium sulfate dihydrate (CaSO<sub>4</sub>.2H<sub>2</sub>O) equal to 7% by weight of the metal-graphite mixture. The mixture may then be compressed or otherwise formed into a block of suitable size to form the desired commutator brush and baked at a temperature of approximately 1,500° F. in a manner well known in the art. The heat treatment converts the calcium sulfate dihydrate (CaSO<sub>4</sub>.2H<sub>2</sub>O) to anhydrous calcium sulfate (CaSO<sub>4</sub>). The heat treatment causes the evaporation of the water held by the calcium sulfate dihydrate (CaSO<sub>4</sub>.2H<sub>2</sub>O).

However, anhydrous calcium sulfate is highly adsorbent of moisture so that upon the graphite block being permitted to cool and the porous block being exposed to moisture carried by the atmosphere water vapor may be adsorbed by the hygroscopic anhydrous calcium sulfate.

Such water vapors are liberated by the latter brush at high altitudes together with oxygen vapors for preventing the dusting of the brush and further causes the formation of an oxide film on the commutator as previously explained.

It has been found that through use of the foregoing invention, the life of commutator brushes at high altitudes in aircraft electrical devices may be remarkably increased.

It is to be understood, however, that the conditions of temperature, concentrations and ingredients disclosed hereinabove are not limitations of my invention, but are to be considered merely as illustrative of the practice thereof, since the invention is not to be limited except by the appended claims.

What is claimed is:

1. A brush for use on a copper commutator, comprising, in combination, a graphite block of

porous structure, said block including therein calcium sulfate, whereby water vapor may be adsorbed within said block for preventing dusting of said brush when in use on said commutator.

5. An article comprising a porous graphite block, and a moisture adsorbent of calcium sulfate.

10. In a method for forming a moisture adsorbent article; the steps consisting in mixing dihydrate calcium sulfate in a porous metal graphite mixture including copper and carbon, compressing said mixture, and then subjecting said mixture to a temperature sufficient to evaporate water from the dihydrate calcium sulfate so as to form anhydrous calcium sulfate, whereby the same is conditioned for the adsorption of atmospheric moisture vapor.

15. In a method for forming a moisture adsorbent article; the steps consisting in mixing barium nitrate in a metal graphite mixture including copper and carbon; compressing said mixture, and then subjecting said mixture to a temperature sufficient to release nitrogen gas from the barium nitrate and cause the formation of barium oxide, and passing such nitrogen gases through said mixture so as to form said graphite mixture into a porous structure, whereby the same is conditioned for the adsorption of atmospheric moisture vapor.

20. 30. 5. A mixture for forming a moisture adsorbent graphite article, comprising in a graphite mixture an ingredient including a hydrated metallic sulfate in which the water is releasable in a vaporous form in response to heat, and said hydrated metallic sulfate being converted into an anhydrous form so as to function as a moisture adsorption agent by such release of said water vapor.

25. 40. 6. An electrical current conducting brush comprising a block of porous material containing a mixture of graphite and a hygroscopic barium oxide derived during the processing of said brush from barium nitrate, and said mixture having such a porosity as to adsorb moisture under high moisture conditions and retain such moisture for low moisture conditions so as to prevent the dusting of said brush at high altitudes.

45. 55. 7. An electrical current conducting brush comprising a block of porous material containing a mixture of graphite and a hygroscopic metallic oxide derived during the processing of said brush from barium nitrate, and said mixture having such a porosity as to adsorb moisture under high moisture conditions and retain such moisture for low moisture conditions so as to prevent the dusting of said brush at high altitudes.

60. 65. 8. An electrical current conducting brush comprising a block of porous material containing a mixture of graphite and a hygroscopic calcium sulfate derived during the processing of said brush from a dihydrated calcium sulfate, and said mixture having such a porosity as to adsorb moisture under high moisture conditions and retain such moisture for low moisture conditions so as to prevent the dusting of said brush at high altitudes.

70. 75. 9. In a method for forming a moisture adsorbent current conducting brush; the steps consisting of adding to a carbon-copper mixture a minor proportion of an inorganic material, said inorganic material being a member of a group consisting of barium nitrate and calcium sulfate dihydrate, then compressing said mixture into the form of a block, baking said block at a temperature sufficient to release a gaseous medium from

2,462,055

5

the inorganic material and change said inorganic material into a hygroscopic form, and passing said gaseous medium through said block so as to form said block into a porous structure, whereby the same is conditioned for the adsorption of atmospheric moisture vapor through capillary action.

10. The method defined by claim 9 in which the proportion of said inorganic material is equal to approximately seven per cent by weight of the carbon-copper mixture, and the baking temperature is approximately 1500 degrees Fahrenheit.

ROBERT S. HERWIG.

**6  
REFERENCES CITED**

The following references are of record in the file of this patent:

**UNITED STATES PATENTS**

| Number    | Name   | Date          |
|-----------|--------|---------------|
| 656,651   | Markey | Aug. 28, 1900 |
| 1,071,044 | Gilson | Aug. 26, 1913 |
| 1,895,756 | Fuller | Jan. 31, 1933 |
| 2,361,220 | Loftes | Oct. 24, 1944 |

**FOREIGN PATENTS**

| Number  | Country       | Date         |
|---------|---------------|--------------|
| 579,509 | Great Britain | Aug. 6, 1946 |